

Oct. 11, 1927.

1,645,348

J. H. PULLMAN

TEXTILE ROLL

Filed March 31, 1926

*Fig. 1.*



*Fig. 2.*



*Fig. 3.*



*James H. Pullman*

INVENTOR

*Frank J. Nuttall*  
BY  
his ATTORNEY.

## UNITED STATES PATENT OFFICE.

JAMES H. FULLMAN, OF FALL RIVER, MASSACHUSETTS.

## TEXTILE ROLL.

Application filed March 31, 1926. Serial No. 98,640.

My invention relates to textile rolls, and more particularly to top rolls having a yieldable covering composed mainly of cork wood.

Heretofore in the production of rolls for drawing, roving, spinning and various other types of textile machinery, used in the production of threads and yarns, it was long the practice to use leather covered rolls, and to the present day such rolls are very extensively used notwithstanding that rolls having various other materials for the covering thereof have been proposed and in some instances have been used. Rolls have been used in which composition cork alone or composition cork mixed with other substances have been used for the covering material, such covering material or cots having been formed either from strips of composition cork formed of granular cork and a binder, or from blocks of such cork.

In the production of composition cork used for this purpose as well as for other purposes, the cork is first granulated, and the granulated cork thoroughly admixed with a suitable binding solution before being placed within a mould, and subjected to heavy pressure and heat in order to secure not only the desired intimate relation of contiguous cork granules, but to secure the setting of the binder while the cork granules are thus in the desired relation to each other. Owing to conditions of manufacture of this granular composition cork, and to the fact that it is the common practice to use graded cork granules, it is necessary to subject the cork composition during the formation of the slabs to heavy pressure, thus tending to compress the various cork granules and particularly the granules of larger dimensions. The cork granules used for composition cork will rarely be of a dimension greater than about one-eighth of an inch, the granules grading downward from this to very small dimensions, but slightly greater than what is known as cork dust.

The composition cork heretofore used in textile rolls has always been this granular cork product. In actual practice granular cork used as a covering for drawing or other textile rolls has the disadvantages that when the larger sized granules of cork are included in the composition, such granules are subjected to a higher degree of compression than smaller granules mixed therewith, and the resiliency inherent to cork will tend to

cause a varying expansion of the different portions of the mass resulting in a pebbled effect at the surface of the cork. In addition to this, in cutting the cork even though sharp knives be used, there is always a possibility that smaller granules of cork will fleck from the cut surface of the cork and thus cause a pitted surface.

In making drawing rolls with such cork, it is the invariable practice after the covering has been applied to the metallic core or arbor, to carefully grind the surface of the covering with the threefold object of truing up the surface, of bringing the roll to an accurate diameter, and removing surface imperfections such as the pebbled effect above referred to and the surface pits due to the flecking of granules from the surface of the cork. There is always likelihood, however, even with this grinding operation, of dislodging granules of cork at the surface during the finishing operation, and thus produce small depressions or pits. Even though a perfect roll is secured by the grinding operation, with continued use of the roll, wear thereon may cause dislodgement of the surface granules and the development of pits.

It has been proposed to correct the above conditions by using granular cork composition cut from the slab in the direction of the application of pressure to the composition cork when forming the slab, but with such material the surface of the covering still is granular throughout and liable to flecking and pitting.

Furthermore, with cork slabs made by the ordinary methods, the length of rolls which can be made is limited to the thickness of the cork slab, which rarely exceeds one to four inches, owing to the fact that an effective compression of the cork composition cannot be secured with any greater final thickness of the material. Hence the length of the rolls or the length of the operative surface thereof is limited to one to four inches. While with the use of a finer grade of cork granules, I am enabled to produce longer rolls from strips of composition cork, sliced from a slab in a direction transverse to the direction of application of pressure when making the slab, and have gotten very satisfactory results, nevertheless such rolls require great care in every stage of the production of the composition cork and its ap-

lication to the rolls, and considerable difficulty is experienced in securing a satisfactory product.

- With the above conditions in mind I have produced drawing or other textile rolls, having the usual metallic arbors and core, and a resilient covering composed of a non-granular composition cork, the cork of which is in a form to cause substantially each particle thereof to extend at least partially through the entire flexible surface of the roll, and present at the surface of the roll, long, narrow areas extending parallel with or about the axis of the roll.
- These particles may be united without subjecting different particles to a varying degree of compressibility, and offer very large areas to which the binder adheres extending radially and also longitudinally of the rolls.

In the completed rolls made from slabs of such cork, any expansion will be circumferentially or substantially circumferentially of the roll, and not radially thereof, and the large surface area with which the binder contacts, extending radially of the roll, will minimize, if not entirely avoid, possibility of surface flecking or pitting during cutting of the composition cork slab preparatory to forming the surface of the roll, during the finishing operation, in producing the roll, and during a continued use of the roll. Furthermore the manner of producing the slabs from which the cork sheets are cut permits rolls of any desired length to be produced, it being possible to produce rolls as long as thirty inches or more with a substantially uniform resiliency throughout, and having a substantially smooth uniform surface which will ensure uniform quality in the threads or yarn produced in machines equipped with such rolls.

Notwithstanding an almost complete absence of grain in natural cork wood, the surfacing material above referred to, formed of composition cork, has a very decided, long, twisted grain such as is found in many of the harder woods, and in the finished product, this grain extends substantially parallel to the axis of the roll, thus having no effect of causing separation of fluff from the fibrous material being treated, due to a pinching of said material as a result of closing of the material of the cover for the roll upon said fibrous material as pressure is applied upon the material through the roll. Furthermore, this long grain ensures substantial uniformity in the pressure applied to the fibrous material at every point of the roll.

In addition to the foregoing characteristics, likelihood of spoilage of the rolls during their production is minimized, and the wearing qualities of the roll are much enhanced. Furthermore, the grinding incidental to the finishing of the roll is not

accompanied by possibility of the formation of surface flecks or pits.

The invention consists primarily in a textile roll having a resilient covering consisting of composition cork composed of thin cork shavings bonded together, said shavings lying in planes extending substantially radially of the roll and having dimensions causing them to extend at least partially through the resilient covering; and in such other novel features of construction and combination of parts as are hereinafter set forth and described, and more particularly pointed out in the claims hereto appended.

Referring to the drawings,

Fig. 1 is an enlarged view of a long textile roll embodying the invention, broken away and shown partly in section;

Fig. 2 is a view of another form of roll embodying the invention; and

Fig. 3 is a view in perspective of a fragmentary portion of a slab from which the roll cover is sliced.

Like letters refer to like parts throughout the several views.

In the embodiment of the invention shown in the drawings, the metallic portion of the roll and its arbors, is indicated at *a*. This core may be of any desired configuration to adapt the rolls to different types of textile machinery, rolls of two different sizes and forms being shown in the drawings. The length of the cover portion of a roll may vary from about one half an inch to the full length of a slab thirty or more inches, as stated. The resilient cover for the roll is composed of cork shavings known as cork wool *b*, such shavings being thin and varying in length from a quarter of an inch upwardly to any desired length, the width of the shavings ranging from an eighth to a quarter of an inch. The shavings, or cork wool, are intimately mixed with a gelatinous or other flexible binder and are charged within a mould and subjected to a sufficiently heavy pressure to force the various shavings into close intimate relation, so that the subsequent application of heat will firmly bond the shavings together through the setting of the binder. In charging the cork wool or cork shavings into the mould, the major portion of these shavings will assume a flatwise position with relation to each other, so that in the completed product the edges of the separate shavings will be presented towards the opposite sides of the top and the bottom of the slab. This condition is indicated in Fig. 3 of the drawings. The result is that when a sheet of from one-eighth to one-half of an inch is cut from the top or the bottom of the slab, each of the shavings will extend throughout a considerable portion of, if not entirely through, this sheet, with the thin edges thereof exposed at the top and bottom, the length of the shavings being such as to

give a long grained effect to the material of the sheet, which grain is somewhat twisted or entangled as in some of the harder woods, thus giving great tenacity to the material of the sheet.

By reason of the thinness of different particles of the cork wool or shavings, the compaction of the cork composition during the making of the slab from which the sheets are cut, does not result in material compression of the several shavings but in the compression of the mass of such as a whole. As a consequence the sheets cut from the slabs will possess a resiliency approximating that of natural cork and this resiliency will be uniform throughout the sheet, the several shavings not having been so distorted by pressure during the formation of the material of the sheet as to produce unequal stresses in different portions of the mass.

A sheet thus cut from a slab is then cut with the grains of the sheet, or at right angles to the lower edge of the sheet shown in Fig. 3, into strips *c* of the desired width to be wrapped about the metallic portion *a* of the roll. The edges of the strip are then joined preferably by means of a skived joint *d*, the ends being united by means of any suitable cement. The strip *c* while being mounted upon the roll *a* is subjected to pressure from a mould in forming this joint and also to an elevated temperature.

In applying the strip *c* to a roll *a*, it is bonded to the metal of the roll by means of a stratum *e* of adhesive, the heat and pressure ensuring the desired engagement of the strip with the metal of the roll and the setting of the cement stratum *e* and that at the joint *d*.

This manner of forming the strip and applying it to the metallic roll, will cause the grain of the covering to extend longitudinally, or axially, of the roll with narrow edges of the shavings presented outwardly thereof, since the various shavings lie in planes extending substantially radially of the roll. The width of these shavings and the thickness of the strip *c* are such that the shavings will extend in some instances partially and in other instances wholly through the thickness of the strip.

After the strip has thus been applied and bonded to the metallic roll, the outer surface thereof is ground off to bring the finished roll to the desired diameter, give it true cylindrical form and impart the desired finish to the roll. This grinding operation will not tend to raise the grain of the covering and will not be accompanied by any flecking or pitting of the surface of the covering, mainly because of the length and edgewise disposition of the shavings or the grained effect resulting therefrom.

After the roll has been thus ground to the

desired size and finish, it may, if desired, receive a thin superficial coating of shellac or other suitable dressing.

The slabs or cork wool ordinarily are about thirty inches in length, sixteen to twenty inches in width, and of a thickness of about one to one and one-half inches, and the grain of the material of the slab will run with the length thereof. Hence since the strips are cut with the grain, rolls as much as thirty inches in length may be readily made, and if it is desired to increase the length of the slab, rolls of still greater length may be made.

In the use of rolls embodying the invention, the fibrous material being worked in the textile machines will pass transversely to the grain of the covering of composition cork, and this being a long, fine grain, there is no possibility of fluff being picked up by the roll from the fibrous material passing thereunder. Furthermore, there will be a uniform compacting action of the resilient roll with relation to this material.

Cork covered rolls have the advantage that the surfacing material is moisture repellent, and is subject to practically no expansion or contraction as a result of temperature changes. The surfacing material of a roll embodying my invention possesses throughout a degree of resiliency approximating that of natural cork, although unlike natural cork, it has a long and decided grain which precludes any possibility of the development of a pebbled surface during the production of the roll or as a result of prolonged wear of the roll.

Furthermore, any expansion in whole or in part of the composition cork covering after the completion of the roll, will be substantially circumferentially thereof, and thus have a tendency to preserve the finish of the roll both as to its density and as to the preservation of the continuous cylindrical face thereof.

It is not my intention to limit the invention to any particular thickness of the composition cork covering, or any particular formation of the metallic core or length of the covering upon said core, it being apparent that such may be varied to adapt the invention to rolls of different lengths, required in different textile machines, and in the handling of different fibrous materials.

Having described the invention, what I claim as new and desire to have protected by Letters Patent, is:—

1. A textile roll having a resilient covering consisting of composition cork composed of thin cork shavings bonded together, said shavings lying in planes extending substantially radially of the roll and having dimensions causing them to extend at least partially through the resilient covering.

2. A textile roll having a resilient cover-

ing consisting of a strip composed of thin cork shavings bonded together, wound about and bonded to a metallic core having arbors in a manner to cause the shavings to extend axially of the roll with the sides thereof lying in planes extending substantially radially thereof, and having the ends thereof bonded together, the thickness of said strip being such that the shavings will extend at least partially through the resilient covering.

3. A textile roll having a resilient covering composed of a strip of composition cork sliced from a slab of such cork in the direction of the line of compression when forming the slab, said composition consisting of thin cork shavings bonded together, and the thickness of said strip being such that the shavings will extend at least partially through the resilient covering, said strip being wound about and bonded to a metallic core having arbors, and having the ends thereof bonded together, said strip being wound in the direction of the line of com-

pression when forming the slab, whereby the edges of the shavings are presented outwardly of the roll and extend axially thereof, and the sides of the shavings occupy planes extending substantially radially of the roll. 25

4. A textile roll having a resilient covering 30 consisting of a strip of composition cork composed of thin cork shavings bonded together, wound about and bonded to a metallic core having arbors, said strip being wound in a direction coinciding with the direction 35 of the application of pressure in forming said composition cork, whereby any expansion of the cork will be circumferentially of the roll, and the finished surface thereof will be free from pits or irregularities due to 40 flecking of the composition cork at the surface thereof.

In witness whereof I have hereunto affixed my signature this 25th day of March, 1926.

JAMES H. PULLMAN.